

## [54] HIGH RESOLUTION DEVELOPED COLOR FILM

[76] Inventor: Richard J. Goldberg, 4814 Brandenburg Pl., Tarzana, Calif. 91336

[21] Appl. No.: 914,165

[22] Filed: Jun. 9, 1978

## Related U.S. Application Data

[63] Continuation-in-part of Ser. No. 815,947, Jul. 15, 1977, Pat. No. 4,183,750.

[51] Int. Cl.<sup>3</sup> ..... G03C 5/04

[52] U.S. Cl. ..... 430/8; 430/15; 430/364

[58] Field of Search ..... 96/74, 55, 9, 12, 1.2, 96/75, 7, 8; 428/207

## [56] References Cited

## U.S. PATENT DOCUMENTS

|           |         |                |         |
|-----------|---------|----------------|---------|
| 2,132,154 | 10/1938 | Gaspar         | 96/12   |
| 2,336,243 | 12/1943 | Hanson         | 96/12   |
| 2,439,901 | 4/1948  | Neumann        | 96/12   |
| 3,113,866 | 12/1963 | Land           | 430/141 |
| 3,362,820 | 1/1968  | Hellmig        | 96/9    |
| 3,486,900 | 12/1969 | Tsunoda et al. | 430/171 |
| 3,497,350 | 2/1970  | Yutzy et al.   | 96/74   |
| 3,723,113 | 3/1973  | Goffe          | 96/1 PS |
| 3,734,735 | 5/1973  | Bories         | 96/55   |
| 3,801,314 | 4/1974  | Goffe          | 96/1 PS |
| 3,849,138 | 11/1974 | Wyckoff        | 96/84 R |
| 3,915,709 | 10/1974 | Welch          | 430/8   |
| 4,124,384 | 11/1978 | Centa          | 96/27 R |

## OTHER PUBLICATIONS

Moser et al., Photographic Science and Engineering, vol. 19, No. 4, Jul./Aug., 1975.

Goffe, "Photographic Migration Imaging", Annual Conference of Photographic Scientists & Engineers, May 19, 1970.

Habib et al., "The Diazoype Process", SPSE Symposium on Unconventional Photographic Systems, Paper No. 22, Oct. 1964.

Federal Microfiche Standards, Document No. PB 167,630, Dec. 1965.

Chemical Abstracts, vol. 77, 27424t, 1972.

Bowlby, British Journal of Photography, pp. 51 and 52, Jan. 16, 1976.

Primary Examiner—J. Travis Brown  
Attorney, Agent, or Firm—Marvin Feldman; Stephen E. Feldman

## [57] ABSTRACT

A high resolution developed color film in which the usual color image is given increased sharpness and resolution by the provision of a metallic silver image interdispersed with and proportional in amount to the color present in the top emulsion layer. The portions not containing color are tanned, and the combination of the silver-color top layer with the tanned uncolored portions provides a high degree of resolution. The developed color film is useful in aerial photography, microfilm and microfiche applications.

15 Claims, 9 Drawing Figures





Fig. 1



LEGEND

\* - LATENT IMAGE  
 (AgX) - UNEXPOSED SILVER HALIDE

*Fig. 2*  
 EXPOSURE



LEGEND

(Ag) - METALLIC SILVER  
 (AgX) - UNEXPOSED SILVER HALIDE

*Fig. 3*  
 FIRST DEVELOPER



*Fig. 4*  
REVERSAL BLEACH



*Fig. 5*  
COLOR DEVELOPER



*Fig. 6*  
SILVER REOXIDATION



*Fig. 7*  
RE-EXPOSE

LEGEND

- - TANNED
- Ⓐ - METALLIC SILVER
- Ⓐ<sub>3Y</sub> - REOXIDIZED SILVER
- Ⓜ - MAGENTA
- Ⓒ - CYAN
- Ⓨ - YELLOW

*Fig. 8*  
THIRD DEVELOPER

LEGEND

- - TANNED
- Ⓐ - METALLIC SILVER
- Ⓜ - MAGENTA
- Ⓒ - CYAN
- Ⓨ - YELLOW

*Fig. 9*  
FIX

## HIGH RESOLUTION DEVELOPED COLOR FILM

This present application is a continuation-in-part of pending application, U.S. Ser. No. 815,947, filed July 15, 1977, now U.S. Pat. No. 4,183,750.

## FIELD OF THE INVENTION

This invention relates to developed color film. Specifically this invention relates to a high resolution developed color camera film.

## BACKGROUND OF THE INVENTION

In present day color photography the effect of color is obtained by three or more emulsions that are superimposed on a base with optical filters between the layers of emulsions. The base may be a transparent one such as a sheet of cellulose acetate, or it may be an opaque one such as a sheet of paper. Additional layers may be present such as antihalation layers, etc. Essentially the color is found in, generally, three separate emulsion layers. Each of the unexposed layers contains a light sensitive silver salt or silver halide and some form of coloring material that is originally substantially colorless but which during the processing of the film is converted to a color in proportion to the amount of silver in the silver image.

The nature of the photographic process is such that a color image cannot be any sharper than the original silver image which it replaces and very often the color image loses a certain amount of detail or resolution. Because of the nature of the color process itself, it is difficult to increase the resolution of the color images, but it has been found possible to increase the resolution of the overall image by making use of a thin silver image in conjunction with the color image in the top layer.

In certain technologies requiring high resolution developed film, such as in the aerial and microfiche/microfilm industries, color film did not provide the degree of resolution obtainable with black and white films. Therefore the use of color films in such industries was minimal at best. This was particularly so in color microfiche where fine reproduction of a color object was generally unobtainable.

In the microfiche/microfilm industry, standards such as *Federal Microfiche Standards*, Document No. PB 176 630, Committe on Scientific and Technical Information Federal Council for Science and Technology, 2nd edit., December 1965, dictated that the master film copy from a camera have a minimum resolution of 127 lines/mm at a background density of 0.9 to 1.2.

While such standards were achieved with black and white film, heretofore the art was incapable of achieving resolutions of about 127 lines/mm at 1.6:1 contrast for color film.

Similarly, aerial color photography resolution standards in industry, such as that found in *Kodak Aerial Films and Photographic Plates*, Publication M-61, Book No. 0-87985-037-X, Eastman Kodak Co. (1972) at p. D-28, sets forth the present commercial level for resolution in aerial color film as 100 lines/mm at a contrast of 1.6:1.

Now there is provided by the present invention, a developed color film from a camera, which exhibits a resolution in excess of 100 lines/mm at a contrast of 1.6:1, and also in excess of 127 lines/mm at a similar contrast. Thus the present developed color film now provides a commercially acceptable color microfiche/-

5 microfilm and an improved developed aerial photography film as well.

It is therefore a principal object of this invention to provide a developed color camera film having an improved resolution.

It is a further object of this invention to provide a developed film as aforesaid wherein the degree of resolution renders the film useful in both microfiche/microfilm as well as in aerial photography applications.

10 It is still a further object of this invention to provide a color film as aforesaid in which the color rendition is faithful to the colors in the photographed object.

The aforesaid as well as other objects and advantages as will become apparent from a reading of this specification, the adjoined claims, and the drawings in which:

15 FIG. 1 is a flow-chart showing the steps in the production of a high resolution color image using a reversal process;

20 FIG. 2 is a fragmentary cross-sectional view, to an enlarged scale, of a section of film immediately after exposure and before any processing has occurred;

25 FIG. 3 is an enlarged fragmentary view similar to FIG. 2 showing the condition of the emulsions of the film after the first development has occurred;

FIG. 4 is an enlarged fragmentary view similar to FIG. 2 showing the condition of the emulsions after the reversal bleach step has been completed;

30 FIG. 5 is an enlarged fragmentary view of the emulsions similar to FIG. 2 showing the condition of the emulsions after the completion of color development;

FIG. 6 is an enlarged fragmentary view similar to FIG. 2 and showing the condition of the emulsions after the completion of the silver re-oxidation step;

35 FIG. 7 is an enlarged fragmentary view of a portion of the emulsions after the film has been re-exposed by light during the processing;

FIG. 8 is a view similar to FIG. 2 showing the condition of the emulsions after the completion of the third development; and

40 FIG. 9 is an enlarged fragmentary view similar to FIG. 2 showing the condition of the three emulsions after the final fixing has been completed.

Broadly speaking this invention relates to a developed color camera film which comprises a substrate or base, a plurality of superimposed layers comprising color images, on the base; and wherein said film has a resolution in excess of 100 lines/mm at a contrast of 1.6:1.

45 In a more specific aspect this present invention is a developed color camera film which comprises;

a base;

50 a plurality of superimposed layers comprising color images, on said base; and

55 a silver image in association with the outermost color image whereby said outermost color-silver image is the sharpest of said images, whereby said film has a resolution in excess of 100 lines/mm at a contrast 1.6:1.

In another aspect, this present invention recognizes that the non-color portions of the layers are to be tanned whereby the refractive index of the tanned non-color layer portions is different from the color layer portions. This selective tanning in combination with the silver outermost image provides an improved high degree of resolution.

60 It is not uncommon for developed color films of this invention to achieve resolution levels greater than 125 lines/mm to 130 lines/mm at contrasts of 1.6:1.

The color camera film of this invention may be processed as set forth hereinafter.

Considering first FIG. 2 of the drawings there is shown a representation of a cross-section of color film having a transparent base 12 on which are placed a blue sensitive, yellow image emulsion 14, a red sensitive, cyan image emulsion 16, and a green sensitive, magenta image emulsion 18. It is to be understood that the yellow, cyan, and magenta images are not originally present in the film or the emulsions but are formed in the separate emulsions during the processing of the film as hereinafter described. However, for purposes of the present description, the emulsions 14, 16 and 18 will be referred to by the color of the images finally formed therein rather than by the original sensitivity of the separate emulsions.

In all color films considered herein, whether reversal films or color negative or color positive films, it is to be understood that each emulsion layer initially contains a light sensitive silver halide and a color coupler that is initially colorless or of a neutral color, but which is converted to the designated color during the color development process.

In accordance with customary photographic practice, the emulsion layer 14 may be separated from the base 12 by a coating 20 which under certain circumstances may include an antihalation backing, and the emulsion 16 separated from the emulsion 14 by a layer 22, just as the emulsion 18 is separated from the emulsion 16 by a layer 24. It will be understood that the layers 22 and 24 may have colors incorporated in them to act as light filters.

It will be noted that the sequence of the emulsions 14, 16 and 18 upon the base 12 is somewhat different from that customarily associated with subtractive color films, but a film having the particular arrangement shown is presently available from Eastman Kodak Company under the trade designation SO 242. Furthermore, as will hereinafter become apparent, the herein described process for developing color films is applicable to both films having the emulsion sequence shown and the heretofore more common sequence in which the blue sensitive, yellow image layer is located outermost.

In each of FIGS. 2 through 9, a section of the film is shown in which the center section has been illuminated by white light and the two outer sections have not been illuminated. Thus, if a light image is focused on the center of the uppermost surface of emulsion 18, in FIG. 2, the right and left hand portions of emulsions 14, 16 and 18 have not been illuminated or exposed, but the center portion of each of these emulsions has been exposed.

Without going into the theory of the photographic process, it is known that when light strikes a photographic emulsion, the silver halide within that emulsion experiences a subtle change and becomes a latent image. The unexposed silver halide experiences no change and does not become what is usually referred to as a latent image. Because the light which is assumed to be falling upon the central portion of the upper surface of the emulsion 18 is white light, this light will pass through all of the emulsions and expose the magenta, cyan, and yellow emulsions.

As indicated by the legend adjacent FIG. 2, the grains of silver halide that have been exposed to form a latent image are indicated by the stars in the emulsions, and the unexposed grains of silver halide are indicated by the circles enclosing the letters AgX.

Turning now to FIG. 1 of the drawings, there is disclosed a flow-chart of the various steps in the processing of color film as set forth in this invention. This includes certain steps enclosed A and B and numbered 5 6 through 10, and 14 through 19, respectively, that are not found in conventional color film processing. A conventional process is set forth by Eastman Kodak Company in its publication "Manual for Processing of 10 Kodak and Eastman Ektachrome Film Using Kodak Process ME4", wherein the description of the so-called ME4 process is given. In that process, after exposure, the film goes through a pre-hardener and then a neutralizer before being passed into a first developer which is a black and white developer. The film is thereafter 15 passed through a stop bath and then washed. From there the film goes to a color developer, and when the color development is completed, the film then passes through a stop bath and is washed. Thereafter it is bleached, fixed, washed, stabilized and dried.

As is known, the negative silver image formed by the first developer is in the form of metallic silver. The amount of metallic silver depends upon the extent of the exposure, and the metallic silver thus exists in the emulsion, together with the unexposed silver halide. This situation after the first development is indicated in FIG. 3, where it will be seen that the metallic silver is located in the central portion which was exposed to the white light while the unexposed silver halide is in each of the adjacent side sections of all three emulsions.

In the normal ME4 processing, the next step is the treatment of the film by the color developer which has the effect of simultaneously reducing the silver halide and forming a dye, the dye being formed only where the silver halide reduction takes place. Thus, if there is only 35 a slight amount of silver halide at a particular point in the green sensitive magenta emulsion 18, only a slight amount of magenta dye will be formed at that point. On the other hand, if there is a large amount of unreduce silver halide at corresponding points in the cyan and yellow layers, there will be correspondingly greater amounts of the cyan and yellow images formed. In order for the color developer to act on the silver halide so that it may be reduced to metallic silver, the halide must be "fogged" either by exposure to light or by use 40 of a fogging agent in the color developer such as tertiary-butyldiamino-borane (TBAB). See 1970 *British Journal of Photography Annual*, page 219.

At this point, after color development, there will be the metallic silver crystals which were formed as a 50 result of the first development, these crystals not having formed any dye images, and other silver crystals that have been formed during the color development phase of the process which crystals are associated with dye images. The crystals formed by the first development may be considered as comprising the negative image, and the crystals formed by the color development and the associated dye images form the complementary or positive image. The terms "positive", "negative" are relative, and the first image may be a "positive", in which case the color image will be a "negative", but in each case the first image and the color image are complementary to each other.

The film is then run through a stop bath that immediately stops all further development, and is then washed. The film is then bleached in a solution that converts the metallic silver to a silver salt and thereafter this salt is removed by a fixing solution in the customary way. Washing and stabilizing of the film complete the pro-

cess. The result of this procedure is a film having a color image composed entirely of the appropriate dyes and having no silver image at all. This conventional process is diagrammatically illustrated by eliminating steps 6 through 10 and 14 through 19 of the process indicated by the flow-chart of FIG. 1.

The improved process has the metallic silver formed by the first developer removed immediately instead of keeping all of the silver, in either metallic silver or silver halide form, through the color development, step number 11. Thus, in FIG. 1, after the formation of the metallic silver negative image, step 4, that image is removed by a reversal bleach while the unexposed silver halide is not disturbed. The condition of the film at this time is indicated in FIG. 4.

It will be noted that this is an additional treatment, designated by the letter A in FIG. 1, and the added steps therein are steps 6 through 10 that include the steps of washing, reversal bleaching, washing, clearing, and washing again. In addition to removing the metallic silver, the reversal bleach also acts to tan or toughen the emulsion where the silver has been. This is indicated by the shaded areas in FIGS. 4 through 9. This tanning, for reasons not clearly understood, aids in improving the sharpness and resolution of the resulting image.

After washing to remove the clearing solution, the film is processed through the color developer, step 11 as previously described, through the stop and wash steps 12 and 13, at which point the emulsions are in the condition indicated in FIG. 5.

Since the negative silver image has been removed by the reversal bleach step, the silver that is left in association with the positive color image, and which is aligned or in register with the color image, is a positive silver image which darkens or degrades the color image. At this point the second modification of the conventional process occurs. This additional treatment, indicated by the letter B, comprises the steps 14 through 19 and includes the re-oxidation of the metallic silver to form a light-sensitive salt that is present in the emulsions and co-extensive with the dye images. This condition is illustrated in FIG. 6.

After washing the film to remove the solution used to re-oxidize the silver, the film is then re-exposed to provide the latent images as indicated in FIG. 7. If desired, the re-exposure may be accomplished by ultraviolet light, which has the property of not penetrating deeply into the photographic emulsions but instead exposes only the outermost silver halide. Thereafter the film is again developed, as indicated in step 17. This third development of the film is carefully controlled so that only the latent image in the outermost emulsion layer is developed and the images in the second and third layers are substantially unaffected. The reason for this careful control is that the image that has been formed on the outermost layer is the sharpest of all three images and acts to greatly increase the resolution of the film. The images formed in the middle and innermost emulsions are much more diffused because of the scattering of the light in its passage through the emulsions, and consequently, the presence of the other images and the middle and innermost emulsions actually tends to degrade the results that can be obtained by keeping the image only on the outermost layer. It will be realized that it is not always possible in commercial operations to restrict the silver image solely to the outermost layer, though this is the desired condition. So long as the principal silver image is in the outermost layer, the presence of a

much fainter image in a more inward layer will not defeat the superior effect of the principal image.

After development of the film in the third developer to provide the metallic silver image in the outermost layer, leaving unaffected the silver halide in the intermediate and innermost emulsions, the film is passed through a stop bath and washed before passing into a fixing bath, step 20. At this point the various emulsions are indicated in FIG. 9 where each of the emulsions has its own respective color image and in addition the outermost emulsion has a silver image.

The process is completed by the washing, stabilizing, and drying of the film.

While all of the solutions in steps 1 through 5, 11 through 13, and 20 through 23, are substantially the same as those customarily used, the first developer, step 4, and the color developer, step 11, are slightly modified. Thus where the first developer normally has 5.50 grams of hydroquinone per liter and 1.38 grams of sodium thiocyanate per liter, the hydroquinone is increased to 33.5 grams per liter and the sodium thiocyanate is increased to 3.08 grams per liter. The pH is changed from 9.90 to 10.15.

The effects of these changes in the composition of the first developer are to steepen the response curve and also to compress or shorten the shoulder of the response curve.

The effect of the extra hydroquinone is to increase the contrast of the negative image and the effect of the thiocyanate is to decrease the size of the shoulder between the sloping straight line portion of the response curve and the flat maximum response. Both of these features are very desirable for increasing the edge sharpness of the resulting positive image that is later secured by reversal and third development.

The color developer used in step 11 is modified by increasing the amount of citrazinic acid from 1.50 grams to 1.90 grams per liter and the pH is changed from 11.65 to 11.85.

The solutions used in the other steps of the conventional color reversal processing are unchanged. However, it will be recognized that there are certain additional steps, those of Group A and Groups B, that constitute chemical treatment beyond the normal washing.

Thus, in Group A, including steps 6 through 10, the film, in addition to being washed in step 6, is treated in a reversal bleach, step 7, and then washed cleared and washed again. The reversal bleach consists of a well-known bleach formula as follows:

|                                    |           |
|------------------------------------|-----------|
| Water                              | 800 ml    |
| Potassium Dichromate               | 30 g      |
| Water to make                      | 1000 ml   |
| Adjust pH with<br>sulfuric acid to | 1.0 ± 0.2 |

The clearing bath that is used after the reversal bleach is as follows:

|                |         |
|----------------|---------|
| Water          | 800 ml  |
| Sodium Sulfite | 100 g   |
| Water to make  | 1000 ml |
| pH as is       | 10.5    |

The steps in part B, steps 14 through 19 inclusive, include a silver re-oxidation bath, step 14, and a third developer, step 17. The silver re-oxidation, step 14, is

accomplished in a solution that may be compounded as follows:

|                                                                         |                          |
|-------------------------------------------------------------------------|--------------------------|
| Water                                                                   | 800 ml                   |
| Sodium Bromide, Anhydrous                                               | 43.0 g                   |
| Potassium Ferricyanide, Anhydrous                                       | 165.0 g                  |
| Borax (Na <sub>2</sub> B <sub>4</sub> O <sub>7</sub> .H <sub>2</sub> O) | 1.0 g                    |
| Polyethylene Glycol                                                     | 3.6 g                    |
| Sodium Hydroxide or Sulfuric Acid                                       | to adjust pH             |
| Water to pH at 80° F.                                                   | 1.0 liter<br>8.70 ± 0.15 |

It will be recognized that this is the ferricyanide bleach set forth in the Eastman Kodak instructions for the ME4 process mentioned above and the function of the bleach is to convert the metallic silver to a light sensitive silver salt.

The third developer is a so-called soft-working developer compounded as follows:

|                                    |         |
|------------------------------------|---------|
| Water                              | 800 ml  |
| Calgon (Sodium hexametaphosphate)  | 1.0 g   |
| Sodium Sulfite                     | 5.0 g   |
| Metol                              | 7.0 g   |
| Sodium Sulfate                     | 50.0 g  |
| Sodium Bromide                     | 0.25 g  |
| Sodium Carbonate (Mono)            | 10.0 g  |
| Water to make                      | 1000 ml |
| Adjust pH with Sodium Hydroxide to | 10.20   |

The time for each of the various steps and the temperature at which it is to be performed are set out below:

| Processing Step     | Time (Seconds) | Temp. °F.   |
|---------------------|----------------|-------------|
| Prehardener         | 120            | 95 ± 1      |
| Neutralizer         | 60             | 93 ± 2      |
| First Developer     | 155            | 93 ± 1      |
| Stop                | 60             | 93 ± 2      |
| Wash                | 60             | 85 ± 5      |
| Reversal Bleach     | 60             | 75 ± 2      |
| Wash                | 60             | 75 ± 2      |
| Clear               | 60             | 75 ± 2      |
| Wash                | 60             | 85 ± 2      |
| Color Developer     | 255            | 98 ± 1      |
| Stop                | 60             | 93 ± 2      |
| Wash                | 60             | 85 ± 5      |
| Silver Re-oxidation | 60             | 100 ± 5     |
| Wash                | 60             | 85 ± 5      |
| Re Expose           | 5-7            | —           |
| Third Developer     | 22             | 70 ± 1      |
| Stop                | 60             | 93 ± 2      |
| Fix                 | 60             | 100 ± 5     |
| Wash                | 60             | 85 ± 5      |
| Stabilizer          | 60             | Equilibrium |

Re-exposure is accomplished by using a No. 2 Photo-flood Lamp at 18 inches from the emulsion side.

As previously mentioned it is very important to restrict, so far as possible, the development by the third developer to the outermost layer of emulsion, and consequently it will be noted that the temperature of that solution is the coldest of all the solutions and the time of treatment is the shortest of all of the chemical treatments. Furthermore, there is no mechanical agitation of the third developer such as might be provided by jets or spray developing, since it is important that the action of the developer be restricted to the surface of the film,

and the actual movement of the film through the solution causes sufficient agitation.

While the process has been described as being applied to a color reversal film, it will be apparent that the same general results may be obtained in the processing of color negative and color positive films. Thus in processing a color negative where no first developer is used, steps 4 through 9 of the herein-described process may be omitted. In this manner, the normal processing steps 10 are followed through color development and thereafter the film is treated by a stop bath and then washed. The unexposed silver is then removed by a fixing bath and washed, corresponding to steps 20 and 21, and the process of section B is then followed. The result will be a 15 negative color film having a negative silver image in the outermost emulsion layer. If it is decided to make a positive color print, the same general sequence of steps will be followed as set forth for the color negative. From the foregoing it will be seen that a method for 20 processing color film has been provided that is fully capable of achieving the results and securing the advantages heretofore set forth.

It is to be understood that the silver image as shown in FIG. 9, corresponds to the magenta image and is of 25 the same sense as the magenta image. That is to say if the color image is a positive then the silver image is a positive, and wherein the color image is a negative the silver image is a negative. It is also to be borne in mind that the amount of silver present in the outermost layer 30 is directly proportional to the amount of color in the outermost layer, as there is a direct correspondence between the silver and outermost color images.

While the aforescribed film is directed to magenta in the outermost layer, other colors may be in the outermost layer, but it has been found pursuant to the present invention that the silver-magenta combination in the outermost layer provides the best resolution results.

While the invention has been described in detail and with reference to specific embodiments thereof, it will 40 be apparent to one skilled in the art that various changes and modifications can be made therein without departing from the spirit and scope thereof.

What is claimed is:

1. A high resolution developed color camera film comprising:  
a base;  
a plurality of superimposed layers on said base, each layer comprising a color image of the same image sense but differently colored, further comprising a silver image corresponding to the color image in the outermost layer, and wherein the film has a resolution in excess of 125 lines/mm at a contrast of 1.6:1.
2. The film of claim 1, wherein, said resolution is in excess of 130 lines/mm at a contrast of 1.6:1.
3. The film of claim 1, wherein said film is a microfiche.
4. The film of claim 1, wherein the layer outermost from said base is sharper than said other layers.
5. The film of claim 1, further comprising tanned non-color portions of said layers.
6. The film of claim 5, said tanned portions being only in said non-color portions.
7. The film of claim 6, wherein said outermost color image is a magenta image.
8. The film of claim 6, wherein the refractive index of said tanned portions is different from the other portions of said layers.

9. The film of claim 1, wherein said film is an aerial camera film.

10. The film of claim 1, wherein the outermost color image is a positive image and the silver image is a positive image. 5

11. A high resolution developed color camera film comprising;

a base;

a plurality of superimposed layers comprising color images, on said base; and 10

a silver image corresponding to the color image in the layer outermost from said base, said silver and color outermost image being sharper than any of the images in the other layers, whereby said film 15 has a resolution in excess of 100 lines/mm at a contrast of 1.6:1.

12. The film of claim 11, further comprising tanned non-color portions of said layers.

13. The film of claim 12, wherein said resolution is in 20 excess of 130 lines/mm at a contrast of 1.6:1.

14. A high resolution developed color microfiche film comprising;

a base;

a plurality of superimposed layers on said base, each layer comprising a color image of the same image sense but differently colored, further comprising a silver image corresponding to the color image in the outermost layer, and wherein said film has a resolution in excess of the Federal Microfiche Standards, of Document No. PB 167 630, Committee Scientific and Technical Information Federal Council for Science and Technology, 2nd. Edit., December 1965 of a distribution copy having a resolution of at least 90 lines per mm with a background density of 0.9 to 1.2.

15. The film of claim 14, further comprising a silver image corresponding to the color image in the outermost layer, wherein the image of the layer outermost from said base is sharper than the image in said other layers.

\* \* \* \* \*

25

30

35

40

45

50

55

60

65